

1

2,967,105

## PHOTOSENSITIVE SHEET

Robert A. Peters, New York, N.Y., assignor to Stupa Corporation, New York, N.Y., a corporation of New York

No Drawing. Filed Oct. 5, 1955, Ser. No. 538,766

1 Claim. (Cl. 96—88)

This invention relates to a photosensitive sheet on which a positive or a negative reproduction may be formed upon photographic exposure to light of significantly greater intensity than sunlight but which can be exposed to sunlight before or after such high intensity photographic exposure without adverse color change, and to methods of preparing and using such photosensitive sheets.

Heretofore the bromides and iodides of heavy metals such as silver and gold have been the preferred photosensitive materials by reason of their ready decomposition under the influence of light. Ferrocyanide compounds have been employed for blueprints but have required an aqueous development. Certain organic compounds such as diazo materials have been sufficiently sensitive to ultraviolet light to be suitable for office reproductions. These diazo papers have generally had the disadvantage of requiring development under the influence of ammonia gas or equivalent reagent. Altho there have been certain proposals in the patent literature relating to diazo papers which provide prints upon exposure to ultraviolet light and without any kind of development whatsoever, there has been no widespread commercial use of the photographic paper requiring no development.

In accordance with the present invention a photographic image is formed upon a suitably prepared photosensitive sheet under the influence of light having an intensity significantly greater than that of sunlight. After the formation of such photographic image, and without development step it can be handled in a normal manner without being extremely sensitive to fading or other color changes attributable to the action of sunlight. The composition of the photosensitive sheet is such that the photosensitive components are capable of forming two kinds of decomposition products. One of the decomposition products is black or similar dark color and the other decomposition product is white, pale yellow, transparent, and/or otherwise contrasting to the dark color of the other decomposition product. If the photosensitive sheet is designed to provide a negative, so that the decomposition product resulting from the high intensity illumination is dark colored, then the exposure of the photosensitive sheet to sunlight does not bring about the formation of any dark colored material. The negative image resulting from the high intensity exposure can be subjected to sunlight for an indefinite period of time but to the extent that the sunlight brings about any decomposition of the photosensitive components of the negative no fading of the negative results by reason of the substantially white color and/or transparency of the decomposition product from exposure to light of the intensity of sunlight.

In certain embodiments of the present invention the photographic sheet comprises organometallic compounds as the photosensitive component. Under the influence of light, and particularly under the influence of ultraviolet light the chemical bond between a carbon of an organic group and the metal of the organometallic compound and/or the bond between two metal atoms of an or-

2

ganometallic compound containing a plurality of metal atoms is broken. This light-induced breaking of a bond in an organometallic forms reactive fragments which can participate in the formation of decomposition products.

- 5 The composition of the photographic sheet can comprise material tending to form transparent and/or white decomposition products if the rate of photochemical decomposition of the organometallic compound is slow but capable of forming dark colored decomposition products  
10 if the rate of decomposition of the organometallic compound is sufficiently rapid.

In preferred embodiments of the present invention the photographic sheet contains three reactive ingredients, namely, bis(tricyclohexyllead), an organic sulfur compound, and an organic oxygen compound. It is possible that the decomposition product resulting from the high intensity illumination partake of the nature of lead sulfide, a dark colored material. It is possible that the photo decomposition product from low intensity exposure partake of the nature of lead oxide which is of a pale yellow color. However, the beneficial results of the present invention are useful without regard to the correctness of this theoretical explanation of the phenomena.

It has been noted that office reproduction prints or engineering prints should comply with requirements such as:

- 25 (1) Good prints should be obtainable by moderately short exposures of about 10 second. Office print exposures are ordinarily within the range of from 5 seconds (short) to about 30 seconds (long). An exposure of about 2  
30 seconds, altho very short for office reproduction prints, is still of a very much higher order of magnitude than the  $\frac{1}{1000}$  of a second or  $\frac{1}{100}$  of a second or other brief exposure required in motion picture photography.  
(2) The image resulting in the office print should provide sufficient contrast between the dark and light portions that no difficulty would be encountered in reading the print.

(3) Neither the light nor the dark portions of the office print should undergo any change making them less readable after prolonged exposure to sunlight.

(4) The unexposed paper should be sufficiently resistant to aging that periods of the magnitude of six months to a year between manufacture and exposure could cause no significant difficulty.

- 45 An office reproduction paper must not only provide a moderately short exposure, adequate contrast, sunlight stability and storage stability, as respectively outlined previously, but it must provide the office reproduction at a low cost competitive with the diazo reproductions.  
50 Only a single molecule is photochemically decomposed by one quantum of light in the ordinary photochemical decomposition. If the reaction mechanism involves the formation of free radicals, the free radical fragments are capable of participating in a chain reaction providing a  
55 many fold increase in the number of atoms effected by a single quantum of light. Thus a mixture of hydrogen and chlorine may be inert in the dark but exploded by exposure to a small amount of light. The light dissociates the chlorine molecule into chlorine atoms and the chlorine atom is a free radical initiating a chain reaction. Benzoyl peroxide decomposes under the influence of ultraviolet light to form free radicals which can participate in chain reactions.

- 60 Some of the earliest and most detailed work concerning the nature of free radicals and their capacity for bringing about chain reactions resulted from the thermal decomposition of organometallic compounds but there have been few studies of the photochemical decomposition of organometallic compounds.

Bis(tricyclohexyllead) $(C_6H_{12})_3Pb—Pb(C_6H_{12})_3$  is a solid which is somewhat sensitive to sunlight but which

can be stored in subdued light. Earlier workers sometimes called this compound tricyclohexylplumbane.

In the development of the present invention certain novel measurements were made which helped to prove the feasibility of a photographic sheet sensitive only to high intensity light. It is helpful to understand the results of exposing solutions of hexacyclohexyldiplumbane to ultra violet light at various distances from a blueprinting lamp. A saturated solution of hexacyclohexyldiplumbane in cyclohexane was prepared. A series of cuvettes, each containing 4 ml. of the saturated solution, were positioned at various distances from a lamp and were exposed for 30 minutes to a blueprinting lamp of sufficient intensity to be designated as a 60 watt per inch lamp. The sample of solution positioned 8 inches from the lamp underwent a photographic decomposition to form a white precipitate. The sample positioned 7 inches from the lamp formed a precipitate which had a slight gray color. The sample of 4 ml. of the saturated solution in the cuvette positioned 6 inches from the lamp underwent a decomposition resulting in a dark brown precipitate. A conspicuously black precipitate formed in the sample positioned 5 inches from the lamp. There appeared to be crystals of metallic lead in the precipitate in the cuvette positioned one inch from the lamp. These prolonged exposures of the solution of the organometallic compound to high intensity ultraviolet light demonstrated not merely that the color of the decomposition product was dependent upon the intensity of light but also that a very great change of color resulted from a relatively small change in the intensity of light within what can be designated the critical range of intensity. Thus the intensity at 6 inches was only about 6% or 178% of the intensity at 8 inches. These novel measurements made it appropriate to formulate the goal of an office reproduction paper which would form white decomposition products upon prolonged exposure to ultraviolet light content of bright sunlight but which would form dark colored decomposition products upon short exposure to an ultraviolet lamp providing an intensity from about 2 to 10 times the ultraviolet intensity of sunlight.

In the development of the present invention, it was established that not only did hexacyclohexyldiplumbane possess a color change depending upon the intensity of illumination but that the compositions containing components capable of reacting with the decomposition product possessed the outstanding advantage of undergoing a different kind of photochemical decomposition under high intensity illumination than under low intensity illumination.

Sunlight does not contain significant amounts of light of X-ray wave length but it does contain significant amounts of ultraviolet light. Most materials which are sensitive to ultraviolet light are not suitable for use in photographic materials by reason of their sensitivity to sunlight. The relatively low intensity of the ultraviolet light of sunlight can have effect on most photosensitive materials over a very long period of time which is very similar to the effect of exposure to a blueprinting lamp or other high intensity ultraviolet source for a typical exposure period such as from 2 to 30 seconds. The phenomena of forming decomposition products of different colors according to whether the light intensity is merely of the order of bright sunlight or significantly greater makes it possible to prepare office prints which do not fade after prolonged exposure to sunlight, notwithstanding the absence of any conventional developing step or fixing step.

Reference is made to a series of examples illustrating some of the chemistry and physics pertinent to the present invention.

#### EXAMPLE I

Hexacyclohexyldiplumbane was prepared by a method substantially the same as that of Krause, Ber., 54, 2060

(1921). A stirred mixture of magnesium turnings in 400 ml. of dry ethyl ether was reacted with 163 g. (1 mol) of cyclohexylbromide. The Grignard solution of bromomagnesiumcyclohexane then was slowly added to 125 g. (0.45 mol, or a 33% excess) of lead chloride, and thereafter the mixture was heated at reflux for from 4 to 24 hours. After hydrolysis, and evaporation of the ether, the solids were extracted with hot benzene. Hexacyclohexyldiplumbane was recovered from the hot benzene solution by several techniques, such as by precipitation upon cooling of the hot solution. Based upon the consumption of bromocyclohexane, the most expensive reactant, the average yield of hexacyclohexyldiplumbane in a series of successful preparations was greater than 50%.

Instead of using a method characterized by the Grignard reagent cyclohexylmagnesiumbromide, other methods of established value in the preparation of organometallic compounds can be utilized. For example, cyclohexyllithium could be reacted with lead chloride in pentane. The purified hexacyclohexyldiplumbane is a light canary yellow color. Two forms of crystals have been identified under the microscope, one being generally hexagonal plates, and the other being of a short fibrous nature or hair-like tubular crystals. In order to obtain optimum results in photosensitive sheets, it is advantageous to purify the crude product by filtering the boiling benzene solution, distilling to remove about 20% of the benzene of the saturated filtrate, and allowing the thus-prepared supersaturated solution to cool to rapidly deposit high purity crystals.

#### EXAMPLE II

A polyethylene resin was found to have an average molecular weight of about 14,000 as measured by the intrinsic viscosity technique. A coating composition was prepared by mixing about 40 ml. of boiling toluene, 10 g. of said polyethylene, and 10 g. of hexacyclohexyldiplumbane. This coating composition was spread upon about 18.5 square meters of a hard finish paper to provide a dry film of about 1 micron thickness. After the evaporation of the toluene solvent, the coating composition consisted of about equal parts by weight polyethylene and hexacyclohexyldiplumbane. The 1 micron thickness of the coating provided approximately 1.08 g./m.<sup>2</sup> or about 2 pounds per 1000 square yards. The thus prepared photosensitive sheet, when exposed for 10 seconds at a distance of six inches from a blueprinting lamp (60 watts per inch) provided negatives which were dark brown in color. Thus it was established that the combination of a resin and hexacyclohexyldiplumbane provided a photosensitive coating for a sheet having attractive qualities for office and/or engineering prints.

#### EXAMPLE III

The advantageous results of using a paper coated with a mixture of an organometallic compound and a resin are not limited to coatings containing polyethylene. A series of tests were conducted using various resins, and noting the effect of a change in the choice of resin.

A parallel series of tests were conducted using tetraethyllead as the organometallic compound in place of hexacyclohexyldiplumbane. Tetraethyllead contains a relatively higher concentration of lead, and only 2 g. of tetraethyllead (about 28% on an equimolar basis) were used in place of the 10 g. of hexacyclohexyldiplumbane. By reason of the high toxicity of tetraethyllead, this tetraethyllead was first adsorbed into particles of colloidal size silica powder, about 5 g. of silica powder (such as results from vapor phase hydration of silicon tetrachloride) being used to adsorb 2 g. of tetraethyllead. The 7 g. of mixture of tetraethyllead on silica were dispersed in the mixture of 10 g. of resin and 50 ml. of solvent to provide a coating composition.

The thin film of coating composition on paper was al-

lowed to dry thoroughly. The thus prepared photosensitive sheet was exposed for 10 seconds to the ultra-violet light of a blueprinting lamp positioned 6 inches from the paper. The results of the tests indicated the color and sunlight stability of the dark portion of the negative. Because the paper was so remote (6 inches) from the lamp, and the intensity was near the lower limit of the critical range, some of the resins effectively inhibited the development of a dark color under these conditions. However these tests provided evidence that under exposure at distances significantly less than 6 inches from the blueprinting lamp some reproduction machines provide an exposure about 1 inch or less from the lamp satisfactorily dark colors would be obtained.

In each case, the 10 g. of resin and the organolead compound were mixed with 50 ml. of solvent consisting of 40 ml. of methyl ethyl ketone and 10 ml. of toluene. After said standard exposure at the 6 inch distance, the various photosensitive papers had colors as indicated in Table 1.

Table 1

| resin                                         | hexacyclohexyldiplumbane |             | tetraethyllead |              |
|-----------------------------------------------|--------------------------|-------------|----------------|--------------|
|                                               | color                    | fading      | color          | fading       |
| polyvinyl chloride                            | dark brown               | very slight | light brown    | slight.      |
| polyvinyl alcohol                             | brown                    | slight      | yellow         |              |
| copoly-PVA-PVC                                | light brown              | some        | do             |              |
| polymethylmethacrylate                        | dark brown               | very slight | dark brown     | Do.          |
| polyethylacrylate                             | do                       | do          | do             | Do.          |
| polybutylacrylate                             | do                       | do          | do             | Do.          |
| polybutylmethacrylate                         | do                       | do          | light brown    | some.        |
| ethyl cellulose                               | brown                    | do          | brown          | Do.          |
| cellulose acetate                             | do                       | some        | light brown    | Do.          |
| cellulose acetobutyrate                       | dark brown               | very slight | do             | Do.          |
| polyacrylonitrile                             | brown                    | some        | brown          | very slight. |
| butylacrylate-cellulose acetobutyrate mixture | very dark brown          | none        | do             | Do.          |
| methyl methacrylate-cellulose acetate mixture | do                       | do          |                |              |

Using an emulsion of methylcellulose in water as the resin for the coating composition made possible the prep-

formulations. Thus the weight of organometallic compound per unit area was approximately 16% as great in the photosensitive sheets using 6 parts of resin to 1 part of photosensitive compound as in the sheets having the 1/1 ratio. Because some of the sheets being tested contained lesser amounts of the photosensitive material, the papers were exposed at a distance of 4 inches from the blueprint lamp. In some instances the exposure was longer than 10 seconds, thus indicating that a commercially satisfactory photosensitive sheet would require relatively larger amounts of activator. The codes assigned to the evaluations of the quality of the resistance to fading of the dark color resulting from the exposure to a high flux of ultra-violet light were: A, excellent; B, good; C, fair; D, noticeable fading; E, troublesome fading; and F, unsatisfactory by reason of fading. Any unsatisfactory discoloration of the white portion of the negative print upon prolonged aging in direct sunlight was coded as sunlight sensitivity or SS. Data relating to selected examples of organo-

metallic compounds as the photosensitive component of photosensitive sheets are set forth in Table 2.

Table 2

| Compound                 | resin to organo-metallic ratio |                      |                   |                    |
|--------------------------|--------------------------------|----------------------|-------------------|--------------------|
|                          | 1/1 p.ethylene color           | 3/1 p.ethylene color | 2/1 PBA-CAB color | 6/1 PBA-CAB color  |
| hexacyclohexyldiplumbane | dark brown, B                  | dark brown, B        | dark brown, B     | dark brown, B.     |
| tetraethyllead           | dark yellow                    | dark yellow          | brown, C          | brown, C.          |
| hexaethylplumbane        | light brown, D                 | light brown          | do                | Do.                |
| tetraphenyllead          | light brown, D60               | light brown, D60     | light brown, B60  | light brown, B60.  |
| hexaphenyldiplumbane     | do                             | do                   | do                | Do.                |
| tetrabutyllead           | dark yellow                    | dark yellow, II      | brown, C          | brown, C.          |
| diphenylead sulfide      | black, A SS                    | black, A SS          | black, A SS       | black, A SS.       |
| tetraphenyltin           | brown, D130                    | brown, D130          | brown, D140       | brown, C140.       |
| tetrabutyltin            | do                             | do                   | do                | Do.                |
| hexabutyltinstanane      | brown, D110                    | brown, D110          | brown, C100       | brown, C100.       |
| hexacyclohexyldistannane | brown, B20                     | brown, B20           | brown, B20        | brown, B20.        |
| dimethyltin sulfide      | do                             | light brown, D20     | light brown, B20  | light brown, B20.  |
| triphenylarsenite        | light brown, D120              | yellow, E120         | yellow, E120      | yellow, C20.       |
| triphenylantimony        | light brown, C120              | yellow, D120         | yellow, D120      | yellow, C20.       |
| tributylantimony         | brown, C100                    | brown, C100          | brown, C100       | light brown, C120. |
| triphenylbismuth         | brown, C30                     | brown, B30           | dark, C20         | brown, C20.        |

aration of a hexacyclohexyldiplumbane paper which had a brown color with a noticeable tendency to fade after exposure. There was a similar tendency for the brown negative resulting from the corresponding photosensitive paper prepared from tetraethyl lead and a water emulsion of methyl cellulose.

## EXAMPLE IV

A series of tests were conducted to determine the effectiveness of various organometallic compounds as photosensitive components in photosensitive sheets. The relative concentration on the organometallic compound on the paper was controlled by regulating the ratio of resin to organo-metallic compound. Polyethylene was the resin used in the 1/1 and 3/1 ratio compositions. The mixture of equal parts of polybutylacrylate and cellulose acetobutyrate was the resin used in the 2/1 and 6/1 ratio

60 advantages are achieved by preparing the photosensitive sheet to include one or more organometallic compounds, each compound containing one or more metals selected from the group consisting of lead, tin, arsenic, antimony and bismuth. Although many of the organometallic compounds of other metals can be decomposed by light of appropriate wave length and intensity, none of such other organometallic compounds demonstrated a highly attractive combination of properties for photosensitive sheets in the tests conducted during the development of the present invention. However, there is reason to believe that organometallic compounds generally possess advantages as photosensitive compounds by reason of the phenomena that the light tends to decompose the metal-metal bond and/or organo-metallic bond preferentially to any decomposition of a carbon-carbon bond in such molecules,

and because the reactive fragments resulting from the photochemical decomposition of an organometallic compound are capable of reacting rapidly in a manner dependent greatly upon the flux or intensity of the ultraviolet light. Certain advantages are achieved by the use of compounds having a metal-metal bond. Certain advantages result from the use of cyclohexyl derivatives. Aromatic derivatives are decomposed by light with greater difficulty. Paraffinic derivatives are of intermediate photosensitivity. Novel measurements were made by taking the spectrograms of solutions of various compounds on a Beckman ultra-violet spectrophotometer. The carbon tetrachloride solutions of a series of organolead compounds were similar in the there was nearly complete transmission for a wide band nearly complete adsorption of a wide band, with a relatively steep curve separating the two zones on the spectrogram. The wave length of 50% transmission provides an important clue to the photosensitivity of an organometallic compound. A significantly shorter ultra-violet wave length characterized tetraphenylead than hexacyclohexyldiplumbane. Tetraethyllead had an intermediate wave length at the point of 50% opacity.

#### EXAMPLE V

The dark color resulting from the photographic exposure may be attributable either to metallic deposit or to a reaction product which is more complex. In the development of the present invention it was established that a variety of sulfur-containing organic compounds served as activators for photographic sheets comprising organo-metallic compounds. It is not known whether the metal forms mercaptides, metal sulfides, or other metal-sulfur type of materials or whether the beneficial effect is attributable to some catalytic or other phenomena. In any event, the photographic sheets containing controlled amounts of activators provide dark colors which are darker, less susceptible to fading, responsive to briefer pe-

5  
10  
15  
20  
25

20  
25

30  
35

cause of the desirability of marketing the photosensitive paper at a cost per square yard lower than the cost of either diazo paper or blueprint (ferrous ferricyanide) paper, it is desirable to use formulations providing an organometallic compound content per 1000 square yards corresponding to less than about one pound of metal. A minimum concentration is equivalent to about 8 ounces per 1000 square yards, and the maximum concentration (if cost is not important) may be about 20 pounds of metal (a correspondingly larger amount of organo-metallic compound) per 1000 square yards.

Comparative experiments on extenders are difficult to interpret. It has been found that the effectiveness of an activator as an accelerator is similar to its effectiveness as an extender. The comparison of the accelerator effectiveness is readily interpreted.

A series of tests were made using the same general formulation, and varying the choice and concentration of the activator. All of the activators listed herein have been shown to be useful in photosensitive sheets, but under the standard comparison tests several of them show varying degrees of sunlight sensitivity. In the sunlight sensitive negative prints, the light color, instead of retaining its initial white color, underwent a darkening when exposed to bright sunlight for a prolonged period of time. The effect of aging, sometimes designated as sunlight sensitivity, is designated in Table 3. A series of papers were prepared by use of compositions consisting of: 10 g. of hexacyclohexyldiplumbane, 5 g. polybutylacrylate, 5 g. toluene (or 20 g. of the stock mixture of these proportions); 10 g. cellulose acetobutyrate, 40 g. methyl ethyl ketone (or 50 g. of a second stock mixture); and the specified amount of the indicated activator. The image was in all cases sufficiently black to be commercially satisfactory, but the exposure time necessary to achieve such result was measured. The data are set forth in Table 3.

Table 3

| activator                            | amount of activator used in composition |                |         |                |                        |                |
|--------------------------------------|-----------------------------------------|----------------|---------|----------------|------------------------|----------------|
|                                      | 0.1 g.                                  |                | 1.0 g.  |                | 10.0 g.                |                |
|                                      | seconds                                 | aging          | seconds | aging          | seconds                | aging          |
| flowers of sulfur.....               | 1                                       | darken.....    | 1       | dark.....      | 1                      | darkens.....   |
| 2-mercapto benzothiazoline.....      | 3                                       | slight.....    | 3       | slight.....    | 2                      | little.....    |
| thiophenol.....                      | 10                                      | yellow.....    | 5       | yellow.....    | 5                      | yellow.....    |
| tetrathium disulfide.....            | 50                                      | v. sl.....     | 30      | slight.....    | 20                     | none.....      |
| potassium ethyl xanthoate.....       | 20                                      | darkens.....   | 10      | browns.....    | 10                     | browns.....    |
| tetrathium tetrathio.....            | 20                                      | slight.....    | 20      | slight.....    | 10                     | slight.....    |
| potassium ethyl xanthoate.....       | 20                                      | darkens.....   | 10      | browns.....    | 10                     | browns.....    |
| thioacetamide.....                   | 20                                      | yellows.....   | 20      | yellows.....   | 20                     | yellows.....   |
| dithiocarbamide.....                 | 30                                      | do.....        | 30      | do.....        | 20                     | Do.....        |
| thiomalic acid.....                  | 30                                      | do.....        | 30      | do.....        | 20                     | Do.....        |
| potassium thiocarbonate.....         | 20                                      | blackens.....  | 20      | blackens.....  | 15                     | blackens.....  |
| phosphorus pentasulfide.....         | 20                                      | do.....        | 20      | do.....        | photo-inflammable..... |                |
| diphenylthiocarbazone.....           | 20                                      | no change..... | 20      | no change..... | 20                     | no change..... |
| thiocemicarbazone.....               | 20                                      | do.....        | 20      | do.....        | 20                     | Do.....        |
| 1,5 diphenyl thiocarbohydrazide..... | 20                                      | yellows.....   | 20      | yellows.....   | 10                     | yellows.....   |

riods of exposure, responsive to lower concentrations of organo-metallic compound per unit area, responsive to lesser intensities of ultra-violet light and/or possessing other advantages over photosensitive sheets without such activators.

Ordinarily the main purpose of including the organic sulfur activators in the composition is for the purpose of reducing the requirements for the organo-metallic compound per unit area, but because the other effects have been established, the term activator is more appropriate than the term extender. Organometallic compounds are generally expensive. Because of this high cost, and be-

65  
70  
75

Extensive experimentation of the type illustrated in Table 3 established that the activator should be a material containing sulfur, selenium or tellurium, and that particular advantages accrued from the use of a material have a functional group selected from the class consisting of  $S^0$ ,  $S=$ ,  $S_n^-$ ,  $SH^-$ ,  $—S—$ ,



which can also be described respectively as elemental sulfur, sulfide and polysulfide, thiol, thioether, thione (comprising also thials and thiocarboxylic groups) and dithiocarboxylic groups.

## EXAMPLE VI

In obtaining a colorless and/or white product from the photo-decomposition of organometallic compounds, the presence of oxygen, peroxides, carbon dioxide, and related materials are especially advantageous. Possibly the reactive fragments resulting from the photochemical decomposition of an organometallic compound have a strong tendency to react relatively slowly with any traces of oxygen or related materials present in the environment, so that this is the predominating reaction except under those conditions in which the rate of photochemical decomposition of the organo-metallic compound is so rapid that free metal and/or metal-sulfur compounds have an opportunity to form.

One of the several methods of obtaining a photosensitive sheet having an overall balance of attractive properties is to coat paper with a composition comprising an organometallic compound, a sulfur-containing activator, and an oxygen-containing inhibitor. The maximum concentration of the activator is desirably not greater than that of the organometallic compound. The optimum concentration of the inhibitor in many compositions is within the range from 1.0 to 10% of the concentration of the activator. The maximum concentration of inhibitor should be less than the organometallic concentration.

In a series of tests, papers were prepared using some of the formulations of Table 3, but adding measured amounts of benzoyl peroxide. The composition was prepared by mixing: a solution consisting of 10 g. of cellulose acetobutyrate, 40 g. of methyl ethyl ketone, the designated amount of the designated activator, and the designated amount of benzoyl peroxide; and 10 g. of hexacyclohexyldiplumbane, 5 g. of polybutylacrylate and 5 g. of toluene. A film about 1 mil thick was formed on paper. The coated paper was exposed to a blueprinting lamp for a sufficient period of time to provide a reasonably black image, and thereafter the stability of the white portions of the negative print to bright sunlight was measured. Data relating to some of these tests are shown in Table 4.

Table 4

| g.   | activator                              | Quantity of Benzoyl Peroxide |             |         |              |         |              |         |              |
|------|----------------------------------------|------------------------------|-------------|---------|--------------|---------|--------------|---------|--------------|
|      |                                        | 10 mg.                       |             | 50 mg.  |              | 100 mg. |              | 200 mg. |              |
|      |                                        | seconds                      | aged color  | seconds | aged color   | seconds | aged color   | seconds | aged color   |
| 0.1  | flowers of sulfur                      | 2                            | light brown | 2       | yellow brown | 2       | yellow brown | 3       | yellow       |
| 1.0  | sulfur                                 | 2                            | black       | 2       | dark brown   | 2       | dark brown   | 3       | yellow brown |
| 10.0 | do                                     | 2                            | do          | 2       | black        | 3       | black        | 3       | brown        |
| 0.1  | 2-mercaptopbenzothiazoline             | 3                            | brown       | 3       | tan          | 3       | yellow       | 3       | white        |
| 1.0  | do                                     | 3                            | do          | 3       | brown        | 5       | tan          | 5       | yellow       |
| 10.0 | do                                     | 2                            | do          | 2       | do           | 3       | yellow       | 5       | pale yellow  |
| 0.1  | potassium ethyl xanthoate              | 20                           | tan         | 5       | tan          | 10      | do           | 20      | white        |
| 1.0  | potassium salt of ethyl xanthoate acid | 10                           | brown       | 10      | brown        | 10      | brown        | 10      | yellow       |
| 10.0 | potassium ethyl xanthoate              | 5                            | do          | 5       | do           | 5       | do           | 10      | brown        |

Some of the other inhibitors which proved to be useful in such photosensitive sheets included lauryl peroxide, tertiary butyl peroxide, urea peroxide, barium peroxide, sodium chlorate, sodium perchlorate, and lead tetraacetate. Other material providing oxygen and/or carbon dioxide might also serve as inhibitors in such compositions.

Because of the desirability of providing a negative print which after indefinite exposure to bright sunlight has a white or pale yellow color contrasting to the dark color, some of the preferred compositions are those illustrated by the use of 200 mg. of benzoyl peroxide in com-

bination with 100 mg. of either 2 mercaptopbenzothiazoline or potassium ethyl xanthoate.

## EXAMPLE VII

5 Although organo-metallic compounds are the preferred embodiments of the present invention, other photosensitive compositions may be employed to achieve the advantageous combination of providing contrasting colors under the influence of light having an intensity greater than sunlight, but not thereafter adversely affected by prolonged exposure to sunlight, notwithstanding the absence of any chemical treatment for fixing and/or developing.

10 A positive paper is prepared by coating a paper with 15 a composition consisting of 10 parts of polybutylacrylate, 10 parts of cellulose acetobutyrate, 5 parts of copper acetylide, and 5 parts of succinyl azide, and 75 parts of tetrahydrofuran. The paper is coated in the dark. The paper is loaded into an ordinary camera, and the picture 20 is taken using three times the number of flash bulbs conventionally used. The intense light decomposes the succinyl azide component of the photosensitive sheet, providing reactive fragments combining with the copper to 25 form a white background material for the white portions of the print. The sheet is then removed from the camera, and the effect of the sunlight on the balance of the print is to form a black copper image. The sunlight brings about the decomposition of the copper acetylide except in those areas in which the copper succinate 30 binds the copper in a form insensitive to sunlight. Instead of copper acetylide, lead azide, silver acetylide, or related light-sensitive metal compound which can react with a dibasic organic acid or chelating compound to 35 form a white compound insensitive to sunlight may be employed. Instead of succinyl azide, any light sensitive chelator, such as the azide of ethylenediamine tetraacetic acid may be employed.

40 Obviously various modifications of the invention are possible without departing from the scope of the invention as set forth in the appended claim.

The invention claimed is:

A photosensitive sheet consisting essentially of a strong 65 backing and a photosensitive composition uniformly coated on the backing, said photosensitive composition consisting essentially of: bis(tricyclohexyllead) in a concentration from 8 ounces to 20 pounds per 1000 square yards of photosensitive sheet; an activator in a concentration within the range from 1% to 100% of the concentration of the bis(tricyclohexyllead), said activator being selected from the group consisting of sulfur, organic thiols, organic sulfides, and salts of organic dithio-

**11**

carboxylic acids; and a peroxide in a concentration within the range from 1% to 100% of the activator.

**References Cited in the file of this patent****UNITED STATES PATENTS**

|           |                       |               |
|-----------|-----------------------|---------------|
| 1,880,503 | Sheppard et al. ----- | Oct. 4, 1932  |
| 1,897,843 | Hickman et al. -----  | Feb. 14, 1933 |
| 1,939,232 | Sheppard et al. ----- | Dec. 12, 1933 |
| 1,976,302 | Sheppard et al. ----- | Oct. 9, 1934  |
| 2,057,016 | DeBoer et al. -----   | Oct. 13, 1936 |

|             |                       |               |
|-------------|-----------------------|---------------|
| 2,095,839   | Sheppard et al. ----- | Oct. 12, 1937 |
| 2,219,463   | Yngve -----           | Oct. 29, 1940 |
| 2,414,839   | Schoen -----          | Jan. 28, 1947 |
| 2,441,561   | Chalkley -----        | May 18, 1948  |
| 5 2,683,643 | Baumann et al. -----  | July 13, 1954 |
| 2,703,283   | Eggert -----          | Mar. 1, 1955  |
| 2,712,996   | Elliot -----          | July 12, 1955 |

**12**

|                       |               |
|-----------------------|---------------|
| Sheppard et al. ----- | Oct. 12, 1937 |
| Yngve -----           | Oct. 29, 1940 |
| Schoen -----          | Jan. 28, 1947 |
| Chalkley -----        | May 18, 1948  |
| Baumann et al. -----  | July 13, 1954 |
| Eggert -----          | Mar. 1, 1955  |
| Elliot -----          | July 12, 1955 |

**OTHER REFERENCES**

10 Coates: Organo-Metallic Compounds, John Wiley, N.Y. (1956), page 141.